

## UNITED STATES PATENT OFFICE

AMBROSE J. MANDELL, OF WESTFIELD, NEW JERSEY

## ELECTRODE AND CONTACT ELEMENT

No Drawing.

Application filed May 19, 1925. Serial No. 31,458.

This invention relates to electrode and contact elements which are subject to electric arcs, such as the contact elements of timing devices and circuit making and breaking devices and the electrodes of spark plugs.

Heretofore the most satisfactory materials obtainable for the manufacture of such elements were platinum and alloys of platinum with other metals of the platinum group. The extremely high cost and scarcity of such metals render their use prohibitive on any large scale. Among the base metals, tungsten is fairly satisfactory for contact points but is altogether unsatisfactory for spark plug electrodes because it oxidizes very rapidly at even moderately high temperatures and is also quite expensive in the ductile condition. The spark plug electrodes have been heretofore commonly manufactured from pure nickel, various alloys of nickel and manganese, and Monel, which is an alloy of nickel, copper, manganese and iron. These materials have been fairly satisfactory heretofore but with the development of the modern high speed internal combustion motor, the service conditions have become more and more severe, so that the necessity of a better electrode material has been imperative.

Among the qualities, which are desirable in an alloy for such elements, the following may be mentioned:—

1. Ability to withstand the cutting and abrading action of an electric spark or high voltage arc, while the metal is at a high temperature.

2. Resistance to oxidation at high temperatures, and to corrosion by products of combustion.

3. Ability to withstand deterioration by changes in internal structure under the conditions of service, so that the electrode does not become brittle, but remains tough and ductile.

4. High thermal conductivity and high or fairly high electrical conductivity.

5. Small tendency to absorb carbon under the service conditions or ability to remain strong and tough whether or not carbon is absorbed.

6. Sufficient strength, toughness, mallea-

bility, and ductility to allow working into the finished form by ordinary methods, and hardness not too great to allow easy machining of the finished material.

I have discovered that by the addition of suitable proportions of silicon or silicon and certain other elements to nickel, an element may be produced which exhibits far greater durability in such service than any other base metal alloy previously known.

Increased ability to withstand the cutting and abrading action of the spark is conferred upon nickel by additions which increase the hardness and strength at high temperatures, and the resistance to oxidation. Not all additions which produce this effect are suitable, however, because many of them have a bad effect upon the other properties, such as thermal and electrical conductivity, ductility, etc. Even small additions of silicon have a powerful hardening effect, and greatly promote the resistance to oxidation, and these effects are retained at high temperatures.

Additions of chromium and tungsten will harden nickel, but in order to produce the effect of a given addition of silicon, so much more chromium or tungsten must be added that the thermal conductivity of the resultant alloy is lowered very much more, and the electrical resistance is very much increased. This effect is so pronounced that the usefulness of the alloys is practically destroyed.

Aluminum has a similar effect in hardening nickel and promoting resistance to oxidation, but the accompanying bad effects are not so pronounced as for chromium or tungsten. The hardening effect of zirconium is great, but the resistance to oxidation obtained by addition of zirconium is not so high, and the high cost of zirconium is a great disadvantage. The same remarks apply to titanium and vanadium. Therefore, while small amounts of any or all of these metals may be added, to the alloy, amounts to be added must not be excessive, and they will not serve to replace all of the silicon. If sufficient silicon is present, none of these metals need be added.

Addition to nickel of sufficient silicon, or of

silicon plus the other metals mentioned, to produce the required resistance to cutting and abrasion, to oxidation, and to deterioration of structure at high temperatures will lower the ductility and toughness considerably, as compared to pure nickel. These latter qualities can be greatly improved by the further addition to the alloy of a suitable proportion of manganese, without harm to the previously mentioned qualities, and this effect of the manganese is so valuable that while manganese is not an absolutely essential constituent, the alloys containing a certain amount of manganese are decidedly preferable to those which contain no manganese, or only trifling amounts. Too much manganese should not be added, as it will cause a lowering of the thermal conductivity, and thereby automatically raise the operating temperature of the electrodes when in service, which will of course mean increased severity of the working conditions and consequently a shorter life.

Metals such as copper and iron should not be present if they can be avoided. These metals are of little or no value in promoting the desirable qualities, and they will reduce the thermal conductivity markedly if more than trifling amounts are present. Iron also has the bad effect in these alloys of reducing the resistance to oxidation, and when much is present, of causing brittleness, nullifying the beneficial effect of the manganese addition.

35 The percentages of the various constituents of the alloy which have been found by experiment to be preferable and desirable are the following:—

Silicon should be present in amounts preferably not to exceed approximately 6 to 7%. Above these percentages the alloy becomes so hard as to be practically unworkable by ordinary methods, which of course destroys its usefulness for this purpose, although in castings, much larger amounts might be used. The preferable addition is from 3 to 5% in which range the alloy is strong, quite tough and ductile, and exhibits all the good qualities previously enumerated. Addition of silicon in amounts less than three per cent is of very marked benefit, but with the smaller additions the benefit to be obtained is of course also less.

Manganese should preferably be present in amounts of approximately 2%, and not greatly to exceed approximately 5%. The beneficial effect on the toughness and ductility of an addition of manganese is very marked, but if more than about 5% is present the thermal conductivity is lowered considerably, without compensating increase of toughness and ductility. If less than about  $\frac{3}{4}$  of 1% or so is present, the effect is small, while with additions of about 2%, the beneficial effects are very pronounced, without any marked de-

crease in thermal or electrical conductivity, as compared with alloys containing little or no manganese.

Any or all of the elements, aluminum, chromium, tungsten, zirconium, titanium, and vanadium may be used to replace a portion of the silicon, but they should not be used to replace all or a major portion of the silicon. Their combined total should not exceed the total of the silicon present, and the total of these elements plus the silicon should not much exceed the 7% mentioned as the practical limit for silicon, for although their effects on the ductility are less, their effects on the thermal conductivity and electrical resistance are greater.

Iron is of no benefit to the alloy, and should be kept as low as possible, because of its bad effects on the resistance to oxidation, the toughness and the thermal and electrical conductivities. It should preferably be present only in such amounts as are unavoidable when working with commercial materials.

The bad effects of copper are much less pronounced, but as copper is of no benefit, it also should be kept as low as possible.

Elements such as sulphur, carbon, phosphorus, etc., should be kept as low as possible, because of their bad effects on the mechanical properties.

The balance of the alloy should be nickel. I am aware that cobalt may be substituted for nickel in this alloy, but the high price of cobalt, as compared with that of nickel makes it, at the present time, an undesirable substitute for nickel, and it offers no compensating advantage over nickel. When nickel is used, the amount of cobalt present should be small, and when cobalt is used, the amount of nickel present should be small, for when large amounts of these elements are present simultaneously, the thermal and electrical conductivities of the resultant alloy are considerably lowered, which is an undesirable effect.

Commercial nickel frequently contains a small amount of silicon, usually less than  $\frac{1}{4}$  of 1 percent, and it is necessary to add additional silicon to the commercial nickel so that the silicon content will be at least  $\frac{1}{2}$  of 1 percent or more.

It will be understood that by the term nickel, I intend cobalt to be considered as an equivalent substitute and that the electrode and contact elements are formed of an alloy of nickel with an added quantity of silicon and preferably also manganese with optionally the addition of small quantities of other substances, all as specified in the appended claims.

It will be obvious that the specific instances, which have been given herein, are intended solely for the purpose of explaining the nature of the invention, and that, therefore, various changes in the details and pro-

portions may be made by those skilled in the art within the principle and scope of the invention, as expressed in the appended claims.

5 I claim:—

1. Electrode and contact elements subject to electric arcs, such as for timing devices, spark plugs, and circuit making and breaking devices, said elements being formed of an alloy comprising a base of nickel with an added quantity of substances selected from the group consisting of silicon, aluminum, chromium, tungsten, zirconium, titanium, manganese, and vanadium, the substances added from said group including at least silicon, and constituting between 1 and 5% of the alloy. 70
- 10 2. Electrode and contact elements subject to electric arcs, such as for timing devices, spark plugs, and circuit making and breaking devices, said elements being formed of an alloy comprising a base of nickel with an added quantity of substances selected from the group consisting of silicon, aluminum, chromium, tungsten, zirconium, titanium, manganese, and vanadium, the substances added from said group including at least silicon, the silicon constituting at least 40% of the added substances. 80
- 15 3. Electrode and contact elements subject to electric arcs, such as for timing devices, spark plugs, and circuit making and breaking devices, said elements being formed of an alloy comprising a base of nickel with an added quantity of substances selected from the group consisting of silicon, aluminum, chromium, tungsten, zirconium, titanium, manganese, and vanadium, the substances added from said group including at least silicon, and constituting less than 10% of the alloy. 90
- 20 4. Electrode and contact elements subject to electric arcs, such as for timing devices, spark plugs, and circuit making and breaking devices, said elements being formed of an alloy comprising a base selected from the group comprising nickel and cobalt with an added quantity of silicon in an amount between 2 to 5%. 100
- 25 5. Electrode and contact elements subject to electric arcs, such as for timing devices, spark plugs, and circuit making and breaking devices, said elements being formed of an alloy comprising a base selected from the group comprising nickel and cobalt with an added quantity of silicon and manganese, the silicon addition varying between  $\frac{1}{2}$  of 1% and 10%, and the manganese varying between nothing and 5%. 110
- 30 6. Electrode and contact elements subject to electric arcs, such as for timing devices, spark plugs, and circuit making and breaking devices, said elements being formed of an alloy comprising a base selected from the group comprising nickel and cobalt with an 115
- 35 120
- 40 125
- 45 130

added quantity of from 3 to 5% silicon and 1 to 5% of manganese.

In witness whereof, I hereunto subscribe my signature.

AMBROSE J. MANDELL.

70

75

80

85

90

95

100

105

110

115

120

125

130